

Jan. 10, 1939.

R. E. FRICKEY

2,143,347

## RAIL HARDENING METHOD AND APPARATUS

Filed July 27, 1936



FIG. 4.

BY

Royal E. Frickey INVENTOR.

Paul D. Lehr

ATTORNEY.

## UNITED STATES PATENT OFFICE

2,143,347

## RAIL HARDENING METHOD AND APPARATUS

Royal E. Frickey, San Francisco, Calif., assignor  
to Welding Service, Inc., San Francisco, Calif.,  
a corporation of California

Application July 27, 1936, Serial No. 92,716

9 Claims. (Cl. 148—21)

This invention relates generally to methods and apparatus for the treatment of railroad rails, to effect hardening of the ends of rail sections.

In Frickey et al., Patent No. 2,013,461, there is disclosed a rail treatment method making use of a heating operation, followed by a chilling or quenching operation. Heating is confined to the localized area at one end of a rail or rail section, to heat an upper layer of metal in the rail ball 5 above the so-called critical temperature, as for example a temperature of about 1500° F. Chilling is carried out by the use of a chilling liquid, such as oil, and by the use of liquid retaining means, whereby virtually a pool or blanket of 10 liquid is applied to the heated area. Chilling is carried out under controlled conditions, whereby when the heating operation is properly controlled, a predetermined degree of hardness is secured which can be duplicated within relative- 15 ly close limits for successive operations.

Hardening of rail ends serves primarily the purpose of minimizing deterioration of rail joints, through pounding of rolling stock upon the rail ends. I have found that rail ends are better 20 able to withstand such deterioration, when the greatest amount of hardening is in a limited zone at the end of the rail, with the remainder of the heat treated area tapering off in hardness, to the hardness of the untreated rail metal, which 25 with ordinary rolled carbon steel rails, is in the neighborhood of 260 Brinell. Excessive hardness at any point in the treated area is apt to cause the metal to become too brittle, with the result that fractures may occur and the metal 30 may break away. Insufficient hardness at the end of the rail will not properly minimize flow of metal under the pounding action of the rolling stock. With an optimum hardness pattern, such as will subsequently be described, I have 35 found that the metal at the end of the rail can attain a fair degree of hardness, as for example in the neighborhood of 400 Brinell, to afford the results desired. The method and apparatus described in said Patent No. 2,013,461 may not afford the optimum hardness pattern described 40 herein, because the chilling rate of the liquid applied to the heated area of the rail is relatively uniform throughout the area, except for variations in the temperature to which the area is 45 initially heated.

In view of the foregoing, it is an object of the present invention to afford a method and apparatus of the above character, which will make possible an optimum hardness pattern for the 50 ends of rail sections. More specifically the pres-

ent method and apparatus controls the rate with which the chilling liquid absorbs heat from the heated area, whereby the greatest degree of hardness is secured in a limited zone at the end of the rail section.

Further objects of the invention will appear from the following description in which the preferred embodiment of the invention has been set forth in detail, in conjunction with the accompanying drawing.

Referring to the drawing:

Fig. 1 is a side elevational view, showing apparatus incorporating the present invention, and being partly diagrammatic.

Fig. 2 is a cross-sectional detail, taken along the line 2—2 of Fig. 1.

Fig. 3 is an enlarged cross-sectional detail, taken along the line 3—3 of Fig. 1.

Fig. 4 is a diagrammatic view illustrating an optimum hardness pattern.

The representative type of apparatus illustrated in the drawing consists of an open bottomed receptacle or liquid retaining means 10, which is adapted to be seated upon the upper surface of a rail 11. For the purpose of adapting the receptacle to different size rails, its lower portion can include an adapter 12. To effect a proper liquid seal with the upper surface of the rail ball, the lower edge of the adapter 12 is shown provided with a slot or groove 13, to receive a suitable packing 14, such as a packing made of asbestos. Likewise a packing 16 is shown interposed between the adapter 12, and the remainder of the receptacle 10. Communicating with the receptacle 10 there is a pipe 17, for introduction of a chilling liquid, and also a pipe 18, for removal of liquid. Within the receptacle 10, pipe 18 can communicate through the lower end of a stand pipe 19, which is shown provided with a suitable check valve 20.

For the purpose of modifying the chilling effect of the liquid over a part of the heated area, baffle means is provided consisting of a strip of sheet metal 21. When the receptacle 10 is seated upon a rail the metal strip 21 occupies a position in close proximity with the upper surface of the rail ball, as shown in Fig. 3. For convenience it can be suitably secured to the receptacle 10, as for example by having the ends of the metal strip bent upwardly, and inserted within the grooves 13. Ordinarily no effort is made to space the metal strip 21 from the upper face of the ball, although in practice surface irregularities of the rail, and irregularities in the strip of metal, permit substantially the entire area covered by the 55

strip 21 to be contacted with liquid, even though certain points on the strip may be in contact with the rail.

The apparatus utilized in conjunction with container 10, for applying a chilling liquid such as oil, should be such that the chilling liquid can be applied under controlled conditions, to produce the desired predetermined results in successive operations. For example, in general conformance with the disclosure of said Patent No. 2,013,461, liquid can be introduced into pipe 17, from a tank 23, by opening the valve 24. The liquid can be removed from pipe 18, by pump 26, which is shown delivering the liquid through a cooler 27, back to the storage tank 23. Tank 23 can be provided with suitable thermostatically controlled heating means, whereby the liquid permitted to flow from this tank through pipe 17, is maintained at a constant temperature. Operation of valve 24, and also the operation of pump 26, can be correlated through an automatic control, whereby pump 26 is started in operation after a predetermined interval following opening of valve 24, with automatic closing of the valve 24 after a predetermined interval of time, followed by automatic stopping of pump 26. With such features of control it is evident that a liquid is first submitted to the receptacle 10, to blanket the area of the rail ball encompassed by the same, with the chilling liquid. Thereafter chilling liquid is circulated through the container 10, until valve 24 is closed, after which the remaining liquid is pumped out through pipe 18, to terminate the chilling operation.

38 Use of the apparatus described above, in the carrying out of the present method, can be described as follows: An upper area of the rail ball at the end of the rail is heated by suitable means whereby an upper layer of metal in the rail ball 40 attains a temperature substantially above the critical temperature of the rail metal. For example this heating operation can be carried out by rapidly traversing an electric arc over a predetermined area of the rail ball, whereby the 45 heat of the arc is distributed over said area, to effect a penetration of heat (to a temperature above the critical temperature of the metal) to a suitable depth, as for example a depth of about  $\frac{1}{2}$  inch. In practice this area can extend substantially entirely across the width of the rail ball, and for a suitable distance back from the end of the rail, such as a distance of about three inches. This heating is carried out under such controlled conditions that the results can 50 be duplicated in successive operations, within relatively close temperature tolerances. For example when heating electrically, the electric input can be maintained relatively constant, and the heating discontinued after a predetermined 55 amount of electrical power consumption. After such a heating operation, the container 10 is applied to the end of the rail, over the heated area, and a quenching operation is carried out, as described above.

60 In the foregoing, reference has been made to a representative heated area extending back for a distance of about three inches from the end of the rail. Under such conditions it is satisfactory to have the metal strip 21 about an inch and one-quarter wide, and located about one inch from the end of the rail, when the container is seated upon the rail as shown in Fig. 1. Chilling liquid introduced into the container 10 blankets the heated area, to effect a rapid absorption of heat, but for that portion of the heated area covered

by metal strip 21, heat absorption occurs at a materially slower rate, due to a baffling effect, which presumably minimizes convection currents in the liquid pool, and also possibly permits some gas pockets to form between this strip and the heated surface of the rail. In any event it has been found that the use of such baffling means serves to taper off the hardness from a limited zone of greatest hardness at the end of the rail, to the hardness of the untreated rail metal. Thus an optimum hardness pattern such as shown in Fig. 4, can be produced or approximated. In this figure, the initially heated area on the upper surface of the rail ball, has been indicated. Likewise the extent of the baffle in a direction longitudinal of the rail, and the positioning of this baffle with respect to the end of the rail, has been indicated. The optimum hardness pattern is illustrated by curve a, which starts with a hardness of about 400 Brinell for a limited zone near the end of the rail, and then gradually decreases to a hardness of about 260 Brinell, near the end of the heated zone.

It should be understood that an optimum hardness pattern such as shown in Fig. 4, is in part attained or approximated by virtue of a drawing action following the chilling operation. In other words in usual practice the chilling operation is discontinued while there is still sufficient heat in the rail to effect the drawing operation, and thereafter flow of heat back into the chilled area causes the hardness of the metal to be modified. In carrying out such a drawing operation it is evident that modification of the chilling action of the liquid, by use of the baffle means 21, will occasion a greater amount of tempering or drawing, for the areas influenced by its proximity. Generally the baffle means 21 need not be of greater extent because the area remote from the end of the rail which is not covered by the baffle is at a somewhat lower temperature than the metal near the end of the rail, at the time the chilling operation is commenced, due to flow of heat into the body of the rail. Likewise such portions of the heated area tend to be modified to a greater degree by the drawing operation.

I claim:

1. In a method of hardening rail ends, heating an upper layer of metal in the rail ball for an area extending a substantial distance along the length of the rail from the end thereof, and then differentially chilling said area to afford a resulting surface hardness pattern, such that the greatest degree of surface hardness is secured in a limited zone of said area at the end of the rail, while for the remainder of said area the surface hardness decreases to a value comparable to the hardness of the untreated rail metal.

2. In a method of hardening rail ends, heating an upper layer of metal in the rail ball for an area extending a substantial distance along the length of the rail from the end thereof, and then differentially chilling the upper surface of said area to afford a resulting surface hardness pattern such that the greatest degree of surface hardness is secured in a limited zone of said area at the end of the rail, while for the remainder of said area the surface hardness decreases to a value comparable to the hardness of the unheated rail metal, said differential chilling being effected by the use of a fluid which is contacted with the heated area.

3. In a method of hardening rail ends, heating an upper layer of metal in the rail ball for an

area extending a substantial distance along the length of the rail from the end thereof, contacting a chilling liquid with substantially the entire upper surface of the heated area and controlling the chilling effect of the liquid for a certain portion of the heated area, whereby a predetermined hardness pattern is secured for the upper surface of the rail.

4. In a method of hardening rail ends, heating an upper layer of metal in the rail ball for an area extending a substantial distance along the length of the rail from the end thereof, contacting a chilling liquid with substantially the entire upper surface of the heated area, such chilling liquid being applied in a manner as to blanket said area, and then controlling the chilling effect of the liquid in such a manner that in a given period of time more heat is absorbed from a limited zone of said area at the end of the rail, than for the remainder of said area.

5. In rail chilling apparatus of the character described, an open bottom liquid retainer adapted to be seated upon a rail ball at one end of the rail section, means for sealing the lower edges of the retainer with respect to the ball of the rail, whereby liquid introduced into the retainer is caused to blanket a limited area of the rail ball, and means within the retainer for modifying the chilling action of said liquid for certain portions of said area.

6. In rail chilling apparatus of the character described, an open bottom liquid retainer adapted to be seated upon a rail ball at one end of a rail section, means for sealing the lower edges of the retainer with respect to the ball of the rail whereby liquid introduced into the retainer is caused to blanket a limited area of the rail ball, and baffle

means within the retainer for modifying the chilling action of liquid for certain portions of said area.

7. In rail chilling apparatus of the character described, an open bottom liquid retainer adapted to be seated upon a rail ball at one end of a rail section, means for sealing the lower edges of the retainer with respect to the ball of the rail, whereby liquid introduced into the retainer is contacted with a limited area of the rail ball, and baffle means overlying a portion of the surface of said area, said baffle means being spaced from the end of the rail and serving to reduce the rate of chilling effected by the liquid introduced into the retainer for said portion.

8. In rail chilling apparatus of the character described, for application to a rail, after an area of the rail, near the end of the same, has been heated, means for blanketing a limited upper area of the rail ball with a chilling liquid, and baffle means comprising a strip of metal, overlying a portion of said area and in relative close proximity to the same.

9. In rail chilling apparatus of the character described, an open bottom liquid retainer adapted to be seated upon a rail ball at one end of the rail section, means for sealing the lower edges of the retainer with respect to the ball of the rail, whereby liquid introduced into the retainer is contacted with a limited area of the rail ball encompassed by the retainer, and baffle means consisting of a strip of metal extending across the lower face of the retainer and adapted to span the upper surface of the rail ball, said strip of metal being spaced from that end of the retainer adapted to be disposed at the end of the rail.

ROYAL E. FRICKEY.